

United States Patent [19]  
Kania

[11] Patent Number: 4,603,064  
[45] Date of Patent: Jul. 29, 1986

- [54] COLOR PLUS CLEAR COATING METHOD UTILIZING ADDITION INTERPOLYMERS FROM ISOBORNYL (METH)ACRYLATE WHICH CONTAIN ALKOXYSLANE AND/OR ACYLOXYSLANE GROUPS
- [75] Inventor: Charles M. Kania, Tarentum, Pa.
- [73] Assignee: PPG Industries, Inc., Pittsburgh, Pa.
- [21] Appl. No.: 762,356
- [22] Filed: Aug. 5, 1985
- [51] Int. Cl.<sup>4</sup> ..... B05D 3/02
- [52] U.S. Cl. ..... 427/407.1; 427/408; 427/407.2; 427/407.3; 427/409; 427/410; 427/412; 427/412.1
- [58] Field of Search ..... 427/409, 407.1, 410, 427/407.2, 407.3, 412.1, 408

[56] References Cited

U.S. PATENT DOCUMENTS

- 2,992,203 7/1961 Protzman ..... 260/45.5  
3,681,298 8/1972 Hurwitz et al. ..... 260/78.5 R  
3,940,353 2/1976 Martorano ..... 260/22 CB  
4,124,551 11/1978 Mathai et al. ..... 260/23 AR  
4,131,572 12/1978 Brendley, Jr. ..... 260/17 R  
4,286,021 8/1981 Brendley, Jr. ..... 428/413  
4,499,150 2/1985 Dowbenko et al. ..... 428/447  
4,499,151 2/1985 Dowbenko et al. ..... 428/447

4,529,632 7/1985 Fujii et al. ..... 427/409  
4,563,372 1/1986 Kurauchi et al. ..... 427/409

Primary Examiner—Thurman K. Page  
Attorney, Agent, or Firm—Thomas M. Breininger

[57] ABSTRACT

Disclosed is a method of coating a substrate comprising the steps of (a) forming a basecoat by coating the substrate with one or more applications of a pigmented basecoating composition; and (b) thereafter forming a topcoat by coating the basecoat with one or more applications of an essentially clear topcoating composition; wherein the basecoating composition and/or the topcoating composition comprises an addition interpolymer containing at least one silicon atom directly bonded to a hydrolyzable group, which addition interpolymer (vinyl type) is derived from a mixture of copolymerizable ethylenically unsaturated monomers containing an isobornyl group-containing monomer selected from the group consisting of isobornyl methacrylate, isobornyl acrylate and a mixture thereof. The amount of isobornyl group-containing monomer based on the total weight of the mixture of copolymerizable ethylenically unsaturated monomers ranges from 10 percent to 60 percent by weight.

24 Claims, No Drawings

**COLOR PLUS CLEAR COATING METHOD  
UTILIZING ADDITION INTERPOLYMERS FROM  
ISOBORNYL (METH)ACRYLATE WHICH  
CONTAIN ALKOXYSLANE AND/OR  
ACYLOXYSLANE GROUPS**

**BACKGROUND OF THE INVENTION**

A coating system becoming increasingly popular, particularly in the automotive industry, is one known as "color plus clear". In this system the substrate is coated with one or more applications of a pigmented basecoating composition to form a basecoat which thereafter is coated with one or more applications of an essentially clear topcoating composition to form a topcoat.

However, there are several disadvantages with a number of known color plus clear coating systems. After conventional basecoating compositions are applied to the substrate, a rather long period of time, on the order of about 30 minutes or more, may be required between the application of the conventional basecoating composition and the conventional topcoating composition. Such a period is needed to prevent adverse attack by components of the conventional topcoating composition, particularly solvents, on the basecoating composition at the interface of the two, a phenomenon often referred to as strike-in. Strike-in adversely affects the final appearance properties of the coated product. Strike-in is an especially serious problem when metallic-flake pigments are employed in the basecoating composition. Strike-in, among other things, can destroy the desired metallic-flake orientation in the basecoat. Moreover, strike-in can adversely affect the overall clarity and distinctness of image in the resulting cured composite film.

Often, known color plus clear systems based on thermosetting resins require elevated temperatures typically of at least 120 degrees Celsius (degrees C.) for curing. It is desirable to provide color plus clear coating methods which utilize relatively low temperatures, for example, below about 82 degrees C., and preferably ambient temperatures. A number of previous attempts to develop such coating systems resulted in systems which had the disadvantages of being too time consuming and/or energy intensive or resulted in cured films which were deficient in various combinations of physical properties.

In accordance with the present invention, a color plus clear coating system has been developed which can provide an acceptable rate of cure at low or even ambient temperatures and results in coated products in which the films exhibit a surprisingly excellent combination of appearance and physical properties, particularly a surprisingly excellent distinctness of image (DOI). A film having a high degree of distinctness of image when viewed from a direction close to the normal to the surface and under, for example, a light fixture such as a fluorescent light fixture having a cross-hatch grid in front of the bulb, exhibits a reflected image of the lighted fixture in the film which appears clear and sharply distinct and which appears to originate deep in the film.

**SUMMARY OF THE PRESENT INVENTION**

The present invention provides a method of coating a substrate comprising the steps of (a) forming a basecoat by coating the substrate with one or more applications of a pigmented basecoating composition; and (b) there-

after forming a topcoat by coating the basecoat with one or more applications of an essentially clear topcoating composition; wherein the basecoating composition and/or the topcoating composition comprises an addition interpolymer containing at least one silicon atom directly bonded to a hydrolyzable group, which addition interpolymer (vinyl type) is derived from a mixture of copolymerizable ethylenically unsaturated monomers containing an isobornyl group-containing monomer selected from the group consisting of isobornyl methacrylate, isobornyl acrylate and a mixture thereof. The amount of isobornyl group-containing monomer based on the total weight of the mixture of copolymerizable ethylenically unsaturated monomers ranges from 10 percent to 60 percent by weight.

A preferred embodiment of the present invention provides a method for coating a substrate comprising the steps of (a) forming a basecoat by coating the substrate with one or more applications of a pigmented basecoating composition comprising an addition interpolymer containing alkoxy silane moieties and/or acyloxy silane moieties prepared by reaction of a mixture of monomers containing (i) one or more, typically at least two, ethylenically unsaturated monomers which do not contain silicon atoms, hereinafter referred to for convenience as ethylenically unsaturated silicon-free monomers, comprising isobornyl (meth)methacrylate, and (ii) a copolymerizable ethylenically unsaturated alkoxy silane monomer and/or a copolymerizable ethylenically unsaturated acyloxy silane monomer; and (b) thereafter forming a topcoat by coating the basecoat with one or more applications of an essentially clear topcoating composition comprising a film-forming thermoplastic resin and/or film-forming thermosetting resin, hereinafter referred to for convenience as "a film-forming resin", which may be the same or different from the addition interpolymer of the basecoating composition. As used herein "isobornyl (meth)acrylate" for convenience is intended to refer to isobornyl methacrylate and/or isobornyl acrylate.

Another preferred embodiment of the present invention provides a method for coating a substrate comprising the steps of (a) forming a basecoat by coating the substrate with one or more applications of a pigmented basecoating composition comprising a film-forming thermoplastic resin and/or film-forming thermosetting resin, referred to above for convenience as "a film-forming resin," which film forming resin is not an addition interpolymer containing alkoxy silane moieties and/or acyloxy silane moieties prepared by reaction of a mixture of monomers containing components (i) and (ii) referred to above; and (b) thereafter forming a topcoat by coating the basecoat with one or more applications of an essentially clear topcoating composition which does comprise an addition interpolymer containing alkoxy silane moieties and/or acyloxy silane moieties prepared by reaction of a mixture of monomers containing components (i) and (ii) referred to above.

The addition interpolymers suitable for the method of the present invention are a subject of a copending application Ser. No. 762,490 to C. Kania filed even date herewith entitled "Addition Interpolymers From Isobornyl (Meth)acrylate Which Contain Alkoxy silane And/Or Acyloxy silane Groups".

DETAILED DESCRIPTION OF THE  
INVENTION

The basecoating composition and/or topcoating composition containing the addition interpolymer typically is moisture-curable at low temperature, preferably at ambient temperature.

The ethylenically unsaturated silicon-free monomers employed in making the interpolymer contain at least one ethylenic carbon to carbon double bond. The ethylenically unsaturated silicon-free monomers contain isobornyl (meth)acrylate as a comonomer. Moreover, isobornyl (meth)acrylate may be used as the only ethylenically unsaturated silicon-free monomer.

An addition interpolymer suitable for the method of the invention may be prepared by various methods. For example, the addition interpolymer may be prepared by hydrosilylation of an isobornyl group-containing addition interpolymer containing carbon-carbon double bonds with a hydrosilane examples of which hydrosilane include halogenated silanes such as methyltrichlorosilane, trichlorosilane, and phenyl dichlorosilane; alkoxy silanes such as methyltriethoxysilane, methyl-dimethoxysilane, phenyltrimethoxysilane, trimethoxysilane, and triethoxysilane; acyloxy silanes such as methyltriacetoxy silane, phenyltriacetoxy silane, and triacetoxysilane; ketoxyamate silanes such as bis(dimethylcyclohexylketoxymate)methylsilane, and bis(cyclohexylketoxymate)methylsilane; alkenyloxy silanes such as methylisopropenoxy silane, and triisopropenoxy silane; and other silanes such as methyltriethoxysilane, triaminosilane, methyltriaminosilane and triaminosilane. The carbon-carbon double bonds can be incorporated into the addition interpolymer by employing compounds such as allyl compounds examples of which include allyl acrylate and allyl methacrylate. The reaction of the hydrosilane with the isobornyl group-containing addition interpolymer containing carbon-carbon double bonds employs a catalyst of a transition metal complex, examples of which transition metals include platinum, rhodium, cobalt, palladium and nickel. Reference can be made to U.S. Pat. Nos. 4,191,713 and 4,399,261 regarding process conditions for carrying out hydrosilylation reactions.

As indicated above, a preferred addition interpolymer for the method of the invention is formed from at least two components, i.e., one or more ethylenically unsaturated silicon-free monomers and an ethylenically unsaturated compound selected from an alkoxy silane monomer, an acyloxy silane monomer or a mixture thereof. The term "ethylenically unsaturated" is employed in a broad sense and is intended to encompass, for example, vinyl compounds, acrylic compounds and methacrylic compounds. The basic criteria with respect to the ethylenically unsaturated monomer are that it contains at least one ethylenic carbon to carbon double bond, that it is copolymerizable without gelation with the silane monomer component, and that it does not otherwise preclude the utilization of the finished interpolymer.

In addition to isobornyl (meth)acrylate, another ethylenically unsaturated silicon-free monomer can be, and typically is, employed in forming the addition interpolymer. Examples of suitable ethylenically unsaturated silicon-free monomers for preparing the addition interpolymer herein include the alkyl acrylates, such as methyl acrylate, ethyl acrylate, butyl acrylate, propyl acrylate, and 2-ethylhexyl acrylate; the alkyl methacry-

lates, such as methyl methacrylate, butyl methacrylate, 2-ethylhexyl methacrylate, decyl methacrylate, and lauryl methacrylate; and unsaturated nitriles, such as acrylonitrile, methacrylonitrile and ethacrylonitrile. Still other ethylenically unsaturated monomers which can be used include: vinyl aromatic hydrocarbons such as styrene, alpha methyl styrene, and vinyl toluene; vinyl acetate; vinyl chloride; and epoxy functional monomers such as glycidyl methacrylate.

In practice, in order to produce desirable properties in the interpolymer, it is preferred to use combinations of ethylenically unsaturated silicon-free monomers which form hard polymer segments, such as styrene, vinyl toluene and alkyl methacrylates having from 1 to 4 carbon atoms in the alkyl group with monomers which form soft polymer segments, such as the alkyl esters of acrylic or methacrylic acid, the alkyl groups having from 1 to 13 carbon atoms in the case of acrylic esters and from 5 to 16 carbon atoms in the case of methacrylic esters. Illustrative of monomers which form soft polymer segments are ethyl acrylate, butyl acrylate, 2-ethylhexyl acrylate, 2-ethylhexyl methacrylate, decyl methacrylate, and lauryl methacrylate. In addition to the hardening and softening monomers, as previously indicated, other monomers such as vinyl acetate, vinyl chloride, vinyl toluene, and acrylonitrile may be included to achieve specific properties in the interpolymer. The interpolymer is formed from about 50 percent to about 95 percent, preferably from about 70 percent to about 90 percent by weight of the ethylenically unsaturated silicon-free monomers based on the total weight of all monomers utilized for preparing the interpolymer. The amount of isobornyl (meth)acrylate for preparing the addition interpolymer can range from 10 percent to 60 percent by weight based on the total weight of all monomers utilized for preparing the interpolymer and thus includes, for example, the total weight of component (i) the ethylenically unsaturated monomers which do not contain silicon atoms, i.e., the ethylenically unsaturated silicon-free monomers, and component (ii) the copolymerizable ethylenically unsaturated alkoxy silane monomer and/or the copolymerizable ethylenically unsaturated acyloxy silane monomer. Advantages obtainable in cured films from addition interpolymers prepared from less than 10 percent by weight of isobornyl (meth)acrylate, based on the aforesaid total weight of all monomers utilized for preparing the interpolymer, fall off markedly when less than the aforesaid 10 percent by weight of isobornyl (meth)acrylate is utilized. Preferred interpolymers are prepared utilizing from 40 percent to 20 percent by weight of isobornyl (meth)acrylate based on the total weight of all monomers utilized for preparing the interpolymer.

The other component of the addition interpolymer is an organosilane compound, which for preferred addition interpolymers for the method of the invention, is an ethylenically unsaturated alkoxy silane, an ethylenically unsaturated acyloxy silane or a mixture thereof. Alkoxy silanes which can suitably be employed and are preferred are the acrylatoalkoxy silanes, such as gamma-acryloxypropyltrimethoxysilane and gamma-acryloxypropyldimethoxymethylsilane, as well as the methacrylatoalkoxy silanes, such as gamma-methacryloxypropyltrimethoxysilane, gamma-methacryloxypropyldimethoxymethylsilane and gamma-methacryloxypropyltris(2-methoxyethoxy) silane. Among the above listed alkoxy silanes, gamma-methacryloxypropyltrimethoxysilane

is especially preferred because of its greater reactivity. Examples of other alkoxy silanes which may be employed include the vinylalkoxysilanes such as vinyltrimethoxysilane, vinyltriethoxysilane and vinyltris(2-methoxyethoxy)silane. Examples of ethylenically unsaturated acyloxy silanes which may be employed include acrylato-, methacrylato- and vinylacetoxysilanes, such as vinylmethyldiacetoxysilane, acrylatopropyltriacetoxysilane, and methacrylatopropyltriacetoxysilane. The interpolymer is formed from about 10 percent to about 30 percent by weight of the above described ethylenically unsaturated silane monomer based on the total weight of all monomers utilized for preparing the interpolymer.

The preferred addition interpolymer is formed by interpolymerizing the ethylenically unsaturated silicon-free monomers with the ethylenically unsaturated silane monomers in the presence of a vinyl polymerization initiator. The preferred initiators are azo compounds such as, for example, alpha alpha'-azobis(isobutyronitrile); peroxides such as benzoyl peroxide and cumene hydroperoxide; and tertiary butyl peracetate, diisopropyl percarbonate, butyl isopropyl peroxy carbonate and similar compounds. The quantity of initiator employed can be varied considerably; however, in most instances, it is desirable to utilize from about 0.1 to about 10 percent based on the weight of monomer solids. A chain modifying agent or chain transfer agent is ordinarily added to the polymerization mixture. The mercaptans, such as dodecyl mercaptan, tertiary dodecyl mercaptan, octyl mercaptan, hexyl mercaptan and mercaptoalkyl trialkoxysilanes, e.g., 3-mercaptopropyltrimethoxysilane, may be used for this purpose as well as other chain transfer agents such as cyclopentadiene, allyl acetate, allyl carbamate, and mercaptoethanol. The mercaptoalkyl trialkoxysilanes have been found to be especially useful where increased durability is needed. Thus, a mercaptoalkyl trialkoxysilane at a level of 0.5 to 15 parts by weight per 100 parts by weight of monomers previously has been found to increase the durability of a coating based on a silane addition interpolymer.

For certain coatings applications it is preferable that the peak molecular weight, as determined by gel permeation chromatography, of the addition interpolymer when in the pigmented basecoating composition be at least about 2,000, more preferably at least about 10,000. If the peak molecular weight is low, the time required for drying or curing the basecoating composition to a degree at least sufficient to allow application of the topcoating composition without undesirable strike-in may be undesirably long for certain coatings applications. Just one advantage of the method of the invention utilizing the addition interpolymer for the basecoating composition is that the topcoating composition typically can be applied to the basecoat after the basecoat has remained at ambient temperature in atmospheric moisture for a short period of time, sometimes as short as 2 minutes, without, for example, the topcoating composition undesirably striking-in to the basecoat. Often, the peak molecular weight, as determined by gel permeation chromatography, of the addition interpolymer when in the pigmented basecoating composition is in a range of from about 2,500 to about 40,000, preferably from about 10,000 to about 20,000.

On the other hand, if the peak molecular weight of the addition interpolymer of the basecoating composition is high, for example greater than about 20,000, the spray application properties of the composition at a

desirably high solids content may be undesirably affected. However, while a basecoating composition containing the addition interpolymer can be applied by any conventional method such as brushing, dipping, flow coating, roll coating, spraying, etc., an advantage of the method of the present invention is that, where desired, it allows a basecoating composition containing addition interpolymer to be spray applied at a high solids content, i.e., 40 percent by weight total solids, preferably 50 percent by weight total solids and higher, when the basecoating composition has a No. 4 Ford Cup viscosity of about 25 seconds or less. Moreover, conventional spraying techniques and equipment can be utilized.

When the topcoating composition contains an addition interpolymer, the peak molecular weight of the addition interpolymer as determined by gel permeation chromatography typically is at least about 2,000, and often is in a range of from about 2,000 to about 20,000, preferably from about 3,000 to about 15,000, and more preferably from about 4,000 to about 10,000. The peak molecular weight of an addition interpolymer for the topcoating composition typically can be rather low since the degree of cure to prevent, for example, striking-in is not an important consideration with respect to the topcoating composition.

Conventional techniques for applying coating compositions to substrates such as those described previously can be employed to apply the topcoating composition of the present invention. However, spraying is the usual method of application. Moreover, as for the basecoating composition, the method of the invention allows a topcoating composition containing addition interpolymer to be spray applied at a high solids content, i.e., 40 percent by weight total solids, preferably 50 percent by weight total solids and higher, when the topcoating composition has a No. 4 Ford Cup viscosity of about 25 seconds or less.

The polymerization reaction for the mixture of monomers to prepare the addition interpolymer is carried out in an organic solvent medium utilizing conventional solution polymerization procedures which are well known in the addition polymer art as illustrated with particularity in, for example, U.S. Pat. Nos. 2,978,437; 3,079,434 and 3,307,963. Organic solvents which may be utilized in the polymerization of the monomers include virtually any of the organic solvents heretofore employed in preparing conventional acrylic or vinyl polymers such as, for example, alcohols, ketones, aromatic hydrocarbons or mixtures thereof. Illustrative of organic solvents of the above type which may be employed are alcohols such as lower alkanols containing 2 to 4 carbon atoms including ethanol, propanol, isopropanol, and butanol; ether alcohols such as ethylene glycol monoethyl ether, ethylene glycol monobutyl ether, propylene glycol monomethyl ether, and dipropylene glycol monoethyl ether; ketones such as methyl ethyl ketone, methyl N-butyl ketone, and methyl isobutyl ketone; esters such as butyl acetate; and aromatic hydrocarbons such as xylene, toluene, and naphtha.

Choice of the specific ethylenically unsaturated silicon-free monomers and ethylenically unsaturated silane monomers typically is made such that the addition interpolymer has a calculated glass transition temperature (Tg) of at least about 25 degrees C., preferably from about 30 degrees C. to about 120 degrees C. The Tg is calculated using a generally known equation as found, for example, in "Fundamentals Of Acrylics" by W. H. Brendley, Jr., *Paint And Varnish Production*, Vol. 63 No.

7, July, 1973, pages 19-27. If the glass transition temperature of the addition interpolymer is too low, for example less than about 25 degrees C., the physical properties of the cured films for protective coatings applications are adversely affected. Such physical properties include, for example, the gloss retention of the films which is a measure of long term durability, the mar resistance of the films, the abrasion resistance of the films, and the desired hardness of the films for protective coatings applications. It has been found that composite films prepared utilizing the color plus clear method of the invention employing the addition interpolymers having an appropriate level of isobornyl (meth)acrylate as set forth infra in the clear topcoating composition, not only exhibit an excellent degree of 15 hardness, but also provide unexpected superior appearance properties such as excellent gloss and exceptional distinctness of image (DOI).

The addition interpolymers serve as film-forming resins in the color plus clear coating method of the invention. Typically, the basecoating composition, and/or the topcoating composition, contains the addition interpolymer, an effective amount of a cure-promoting catalyst and, for application purposes, often a solvent. The cure-promoting catalyst may be an organic acid, such as, for example, p-toluenesulfonic acid, and n-butylphosphoric acid; a metallic salt of an organic acid, such as, for example, tin naphthenate, tin benzoate, tin octoate, tin butyrate, dibutyltin dilaurate, dibutyltin diacetate, iron stearate, and lead octoate; an organic base, such as, for example, isophorone diamine, methylene dianiline, and imidazole; a compound containing a fluoride ion such as tetrabutyl ammonium fluoride, benzyl trimethyl ammonium fluoride, sodium fluoride, potassium fluoride and cesium fluoride; or a mixture thereof.

The specific amounts of cure-promoting catalyst which are included in the compositions containing the addition interpolymer vary considerably depending upon factors such as the rate of cure desired, the specific composition of the addition interpolymer component, the amount of moisture present in the ambient atmosphere and the like. However, in general, the coating compositions containing addition interpolymer utilized in the method of the invention may contain from about 0.01 part to about 5 parts by weight of cure-promoting catalyst based on 100 parts by weight of interpolymer solids.

In addition to the foregoing components, the coating compositions containing addition interpolymer employed in the method of this invention may contain optional ingredients, including various pigments of the type ordinarily utilized in coatings of this general class. In addition, various fillers; plasticizers; antioxidants; mildewcides and fungicides; surfactants; various flow control agents including, for example, thixotropes and additives for sag resistance and/or pigment orientation based on polymer microparticles (sometimes referred to as microgels) described for example in U.S. Pat. Nos. 4,025,474; 4,055,607; 4,075,141; 4,115,472; 4,147,688; 4,180,489; 4,242,384; 4,268,547; 4,220,679; and 4,290,932 the disclosures of which are hereby incorporated by reference; and other such formulating additives may be employed in some instances. A composition containing the addition interpolymer is ordinarily applied in an organic solvent which may be any solvent or solvent mixture in which the materials employed are compatible and soluble to the desired extent. It has been found

5 previously that a primary thiol, e.g., dodecylmercaptan, isoctylthioglycolate, and the mercaptoalkyl trialkoxysilanes such as gamma-mercaptopropyltrimethoxysilane, when included in a coating composition based on a silane addition interpolymer, enhances the gloss of the 10 cured coating and such components for enhancing gloss optionally may be included in a composition for the method of the present invention. When a primary thiol is utilized in the coating composition a level of about 0.1 part by weight to about 5 parts by weight primary thiol per 100 parts by weight interpolymer provides this enhanced gloss effect. However, it has been found that the method of the invention utilizing topcoating compositions based on the addition interpolymers prepared employing an appropriate level of isobornyl (meth)acrylate can provide films having in addition to excellent durability properties, unexpected excellent appearance properties such as high gloss and exceptional distinctness of image when compared to a color plus clear method utilizing known silane addition interpolymer prepared without employing an effective level of isobornyl (meth)acrylate. Moreover, the benefits with respect to appearance of cured films from the method of the invention, can be obtained without the utilization of such gloss enhancing additives as the aforesaid primary thiols.

20 The method of the invention may be employed utilizing a wide variety of substrates such as wood, metals, glass, cloth, plastics, foams and the like, as well as over primers. The method of the invention is especially useful for coating automobiles, particularly for automobile refinishing.

25 As indicated, the coating compositions containing addition interpolymer can be cured by heating or typically by exposure to atmospheric moisture at ambient temperature. Thus, once the interpolymer component and cure-promoting catalyst component are brought in contact with each other, as by admixing, and exposed to the ambient atmosphere, the composition will begin to 30 cure. Accordingly, it is desirable in some instances to prepare the compositions containing addition interpolymer in the form of a two package system, i.e., one package containing the interpolymer component along with any desired optional ingredients and a second package 35 containing the cure-promoting catalyst component. The addition interpolymer component of the composition in the absence of the cure-promoting catalyst exhibits good pot life, i.e., 6 months or more when stored at temperatures of 120 degrees Fahrenheit (F), i.e., 48.9 degrees C., or less. When it is desired to coat a substrate with the composition of addition interpolymer, the components of the two packages are merely mixed together just prior to application and the resulting composition applied to the substrate by one of the methods 40 such as those described above.

45 As indicated previously, at least one of the basecoating composition and topcoating compositions contains as film-forming resin the addition interpolymer either as the sole film-forming resin or optionally in combination with an additional film-forming thermoplastic and/or thermosetting resin. Examples of such additional film-forming thermoplastic and/or thermosetting resins include the generally known celluloses, acrylics, amino-plastics, urethanes, polyesters, polyethers, epoxies or mixtures thereof. Additionally, when only one of the basecoating and topcoating compositions contains the addition interpolymer, the other contains a film-forming resin typically selected from the generally known cellul-

losics, acrylics, aminoplasts, urethanes, polyesters, epoxies or mixtures thereof mentioned immediately above. These film-forming resins can be employed optionally in combination with various ingredients generally known for use in coating compositions containing film-forming resins of these general classes. Examples of these various ingredients include: fillers; plasticizers; antioxidants; mildewcides and fungicides; surfactants; various flow control agents including, for example, thixotropes and also additives described previously for 10 sag resistance and/or pigment orientation based on polymer microparticles.

Pigments suitable for the pigmented basecoating composition include a wide variety of pigments generally known for use in coating compositions. Suitable 15 pigments include both metallic flake pigments and various white and colored pigments.

Examples of metallic flake pigments include generally known metallic flakes such as aluminum flakes, nickel flakes, tin flakes, silver flakes, chromium flakes, stainless steel flakes, gold flakes, copper flakes and combinations thereof. Of the metallic flake pigments, non-leaving aluminum flakes are preferred.

Examples of white and colored pigments include generally known pigments based on metal oxides; metal hydroxides; metal sulfides; metal sulfates; metal carbonates; carbon black; china clay; phthalo blues and green, organo reds, and other organic dyes.

The Examples which follow are submitted for the purpose of further illustrating the nature of the present 30 invention and should not be regarded as a limitation on the scope thereof.

As used in the body of the specification, examples, and claims, all percents, ratios and parts are by weight unless otherwise specifically indicated. As used herein, "pbw" stands for "parts by weight".

Glass transition temperatures, where given for the acrylic silane addition interpolymers in the following examples, are calculated using the generally known equation as found, for example, in "Fundamentals of Acrylics" by W. H. Brendley, Jr., *Paint and Varnish Production*, Vol. 63 No. 7, July, 1973, pages 19-27. In these calculations values of 110 degrees C. and 125 degrees C. are used for the glass transition temperatures of homopolymers of gamma-methacryloxypropyl trimethoxy silane and isobornyl methacrylate respectively.

#### EXAMPLE 1

The following monomers are used to make an addition 50 interpolymer suitable for the method of the invention:

| Percent by Weight                             |      |
|-----------------------------------------------|------|
| Isobornyl methacrylate                        | 40.0 |
| Butyl methacrylate                            | 20.0 |
| Butyl acrylate                                | 20.0 |
| Gamma-methacryloxy-<br>propyltrimethoxysilane | 20.0 |

A reaction vessel equipped with condenser, stirrer, thermometer and means for maintaining a nitrogen blanket is charged with 428 grams (g) of butyl acetate and heated to reflux, about 125 degrees C., while under a nitrogen blanket and agitation. Three feeds identified herein as A, B, and C are next gradually and simultaneously added to the vessel over a period of two hours while the contents of the vessel are maintained at reflux

conditions. Feed A consists of a mixture of 928 g isobornyl methacrylate, 464 g butyl methacrylate, 464 g butyl acrylate, and 464 g gamma-methacryloxypropyltrimethoxysilane. Feed B consists of a mixture of 254 g of butyl acetate and 116 g 2,2'-azobis-(2-methyl butane nitrile) available as VAZO-67 from E.I. DuPont de Nemours and Company. Feed C consists of 154 g butyl acetate and 116 g gamma-mercaptopropyltrimethoxysilane. After the addition of the three feeds A, B, and C is complete, a mixture of 22 g butyl acetate and 9.28 g of VAZO-67 is added all at once to the vessel and the contents of the vessel held at reflux for 1 hour. Next, another mixture of 22 g butyl acetate and 9.28 g of the VAZO-67 is added all at once to the vessel and the contents of the vessel thereafter held at reflux for an additional 1½ hours after which period heating is discontinued.

The resultant product is an addition interpolymer suitable for the method of the invention.

The resultant product has a theoretical total solids content of 72.5 percent by weight, an experimentally determined total solids content at 110 degrees C. for 1 hour of 71.15 percent by weight, a Gardner Holdt bubble tube viscosity of G-H, a color value of 1, and acid value of 0.1, and a peak molecular weight of the addition interpolymer of 2685 as determined by gel permeation chromatography using a polystyrene standard. Analysis of the resultant product shows a content of butyl methacrylate of 0.49 percent by weight, a content of butyl acrylate of 0.19 percent by weight, and a content of isobornyl methacrylate of 1.16 percent by weight.

#### EXAMPLE 2

This example illustrates the preparation of an addition interpolymer for use in the basecoating composition of Example 9 and in the comparative clearcoating composition G of Example 9.

The following monomers are used to make the addition 35 interpolymer:

| Percent by Weight                             |      |
|-----------------------------------------------|------|
| Methyl methacrylate                           | 40.0 |
| Styrene                                       | 25.0 |
| Butyl acrylate                                | 10.0 |
| Butyl methacrylate                            | 10.0 |
| Gamma-methacryloxy-<br>propyltrimethoxysilane | 15.0 |

A reaction vessel equipped with condenser, stirrer, thermometer and means for maintaining a nitrogen blanket is charged with 336 g of butyl acetate, 144.0 g of VM & P naphtha, and 96.0 g of toluene and heated to reflux, about 125 degrees C., while under a nitrogen blanket and agitation. Three feeds identified herein as A, B, and C are next gradually and simultaneously added to the vessel over a period of two hours while the contents of the vessel are maintained at reflux conditions. Feed A consists of a mixture of 896.0 g 2-ethylhexyl methacrylate, 224.0 g butyl methacrylate, 224.0 g butyl acrylate, 560.0 g styrene, and 336.0 g gamma-methacryloxypropyltrimethoxysilane. Feed B consists of a mixture of 192.0 g of butyl acetate and 112.0 g di-tertiarybutyl peroxide. Feed C consists of 192.0 g butyl acetate and 112.0 g gamma-mercaptopropyl trimethoxysilane. After the addition of the three feeds A, B, and C is complete, 8.96 g of di-tertiarybutyl peroxide

is added all at once to the vessel and the contents of the vessel held at reflux for 1 hour. Next, 8.96 g of the di-tertiarybutyl peroxide is added all at once to the vessel and the contents of the vessel thereafter held at reflux for an additional 1½ hours after which period heating is discontinued and the contents of the vessel allowed to cool to room temperature. The resultant product is a silane addition interpolymer.

The resultant product has a theoretical total solids content of 70 percent by weight, an experimentally determined total solids content at 150 degrees C. for 1 hour of 71.15 percent by weight, a Gardner Holdt bubble tube viscosity of Z-2+, an acid value of 0.09, and a peak molecular weight of the silane addition interpolymer of 7800 and a weight average molecular weight of 10,000 both determined by gel permeation chromatography using a polystyrene standard. Analysis of the resultant product shows an undetectable amount of styrene, a content of butyl methacrylate of 0.09 percent by weight, a content of butyl acrylate of 0.06 percent by weight, and a content of methyl methacrylate of 0.4 percent by weight.

### EXAMPLE 3

The following monomers are used to make an addition interpolymer for the clearcoating composition A of example 10:

|                                           | Percent by Weight |
|-------------------------------------------|-------------------|
| Isobornyl methacrylate                    | 40.0              |
| Butyl methacrylate                        | 20.0              |
| Methyl methacrylate                       | 20.0              |
| Gamma-methacryloxy-propyltrimethoxysilane | 20.0              |

A 4-neck flask equipped with condenser, stirrer, thermometer, 3 dropping funnels, and means for maintaining a nitrogen blanket is charged with 428 g of butyl acetate and heated to reflux, about 125 degrees C., while under a nitrogen blanket and agitation. Three feeds identified herein as A, B, and C are next gradually and simultaneously added to the vessel over a period of two hours while the contents of the vessel are maintained at reflux conditions. Feed A consists of a mixture of 928 g isobornyl methacrylate, 464 g butyl methacrylate, 464 g methyl methacrylate, and 464 g gamma-methacryloxypropyltrimethoxysilane. Feed B consists of a mixture of 254 g of butyl acetate and 116 g 2,2'-azobis-(2-methyl butane nitrile) available as VAZO-67 from E.I. DuPont de Nemours and Company. Feed C consists of 154 g butyl acetate and 116 g gamma-mercaptopropyltrimethoxysilane. After the addition of the three feeds A, B, and C is complete, a mixture of 22 g butyl acetate and 9.28 g VAZO-67 is added all at once to the vessel and the contents of the vessel held at reflux for 1 hour. Next, another mixture of 22 g butyl acetate and 9.28 g of the VAZO-67 is added all at once to the vessel and the contents of the vessel thereafter held at reflux for an additional 1½ hours after which period heating is discontinued and the contents of the vessel allowed to cool to room temperature.

The resultant product is an addition interpolymer suitable for the method of the invention.

The resultant product has a theoretical total solids content of 72.5 percent by weight, an experimentally determined total solids content at 150 degrees C. for 1 hour of 67.4 percent by weight, a viscosity of 8.28 Stokes, an acid value of 0.02, a color value of 1, and a peak molecular weight of the addition interpolymer of 3143 as determined by gel permeation chromatography using a polystyrene standard. Analysis of the resultant product shows a content of butyl methacrylate of 0.62 percent by weight, a content of methyl methacrylate of 0.50 percent by weight, a content of isobornyl methacrylate of 0.69 percent by weight and a content of styrene of 0.03 percent by weight.

hour of 66.0 percent by weight, a Gardner Holdt bubble tube viscosity of S, an acid value of 0, and a peak molecular weight of the addition interpolymer of 2900 as determined by gel permeation chromatography using a polystyrene standard. Analysis of the resultant product shows a content of butyl methacrylate of 0.86 percent by weight, a content of methyl methacrylate of 0.67 percent by weight, and a content of isobornyl methacrylate of 2.60 percent by weight.

### EXAMPLE 4

The following monomers are used to make an addition interpolymer for the clearcoating composition B of Example 9:

|                                           | Percent by Weight |
|-------------------------------------------|-------------------|
| Isobornyl methacrylate                    | 20.0              |
| Styrene                                   | 20.0              |
| Butyl methacrylate                        | 20.0              |
| Methyl methacrylate                       | 20.0              |
| Gamma-methacryloxy-propyltrimethoxysilane | 20.0              |

A 4-neck flask equipped with condenser, stirrer, thermometer, 3 dropping funnels, and means for maintaining a nitrogen blanket is charged with 440.0 g of butyl acetate and heated to reflux, about 125 degrees C., while under a nitrogen blanket and agitation. Three feeds identified herein as A, B, and C are next gradually and simultaneously added to the vessel over a period of two hours while the contents of the vessel are maintained at reflux conditions. Feed A consists of a mixture of 464.0 g isobornyl methacrylate, 464.0 g styrene, 464.0 g butyl methacrylate, 464.0 g methyl methacrylate, and 464.0 g gamma-methacryloxypropyltrimethoxysilane. Feed B consists of a mixture of 264.0 g of butyl acetate and 116 g 2,2'-azobis-(2-methyl butane nitrile) available as VAZO-67 from E.I. DuPont de Nemours and Company. Feed C consists of 132.0 g butyl acetate and 116.0 g gamma-mercaptopropyltrimethoxysilane. After the addition of the three feeds A, B, and C is complete, a mixture of 22 g butyl acetate and 9.28 g VAZO-67 is added all at once to the vessel and the contents of the vessel held at reflux for 1 hour. Next, another mixture of 22 g butyl acetate and 9.28 g of the VAZO-67 is added all at once to the vessel and the contents of the vessel thereafter held at reflux for an additional 1½ hours after which period heating is discontinued and the contents of the vessel allowed to cool to room temperature.

The resultant product is an addition interpolymer suitable for the method of the invention.

The resultant product has a theoretical total solids content of 72.5 percent by weight, an experimentally determined total solids content at 150 degrees C. for 1 hour of 67.4 percent by weight, a viscosity of 8.28 Stokes, an acid value of 0.02, a color value of 1, and a peak molecular weight of the addition interpolymer of 3143 as determined by gel permeation chromatography using a polystyrene standard. Analysis of the resultant product shows a content of butyl methacrylate of 0.62 percent by weight, a content of methyl methacrylate of 0.50 percent by weight, a content of isobornyl methacrylate of 0.69 percent by weight and a content of styrene of 0.03 percent by weight.

## EXAMPLE 5

The following monomers are used to make an addition interpolymer for the clearcoating composition C of Example 9:

|                                           | Percent by Weight |
|-------------------------------------------|-------------------|
| Isobornyl methacrylate                    | 15.0              |
| Styrene                                   | 25.0              |
| Butyl methacrylate                        | 20.0              |
| Methyl methacrylate                       | 20.0              |
| Gamma-methacryloxy-propyltrimethoxysilane | 20.0              |

A 4-neck flask equipped with condenser, stirrer, thermometer, 3 dropping funnels, and means for maintaining a nitrogen blanket is charged with 440.0 g of butyl acetate and heated to reflux, about 125 degrees C., while under a nitrogen blanket and agitation. Three feeds identified herein as A, B, and C are next gradually and simultaneously added to the vessel over a period of two hours while the contents of the vessel are maintained at reflux conditions. Feed A consists of a mixture of 348.0 g isobornyl methacrylate, 580.0 g styrene, 464.0 g butyl methacrylate, 464.0 g methyl methacrylate, and 464.0 g gamma-methacryloxypropyltrimethoxysilane. Feed B consists of a mixture of 264.0 g of butyl acetate and 116 g 2,2'-azobis-(2-methyl butane nitrile) available as VAZO-67 from E.I. DuPont de Nemours and Company. Feed C consists of 132.0 g butyl acetate and 116.0 g gamma-mercaptopropyltrimethoxysilane. After the addition of the three feeds A, B, and C is complete, a mixture of 22 g butyl acetate and 9.28 g VAZO-67 is added all at once to the vessel and the contents of the vessel held at reflux for 1 hour. Next, another mixture of 22 g butyl acetate and 9.28 g of the VAZO-67 is added all at once to the vessel and the contents of the vessel thereafter held at reflux for an additional 1½ hours after which period heating is discontinued and the contents of the vessel allowed to cool to room temperature.

The resultant product is an addition interpolymer suitable for the method of the invention.

The resultant product has a theoretical total solids content of 72.5 percent by weight, an experimentally determined total solids content at 150 degrees C. for 1 hour of 69.5 percent by weight, a viscosity of 11.6 Stokes, an acid value of 0, a color value of 1, and a peak molecular weight of the addition interpolymer of 3386 as determined by gel permeation chromatography using a polystyrene standard. Analysis of the resultant product shows a content of butyl methacrylate of 0.52 percent by weight, a content of isobornyl methacrylate of 0.40 percent by weight and a content of styrene of 0.05 percent by weight.

## EXAMPLE 6

The following monomers are used to make an addition interpolymer for the clearcoating composition D of Example 9:

|                        | Percent by Weight |
|------------------------|-------------------|
| Isobornyl methacrylate | 10.0              |
| Styrene                | 30.0              |
| Butyl methacrylate     | 20.0              |
| Methyl methacrylate    | 20.0              |
| Gamma-methacryloxy-    | 20.0              |

-continued

|                        | Percent by Weight |
|------------------------|-------------------|
| propyltrimethoxysilane | 5                 |

A 4-neck flask equipped with condenser, stirrer, thermometer, 3 dropping funnels, and means for maintaining a nitrogen blanket is charged with 440.0 g of butyl acetate and heated to reflux, about 125 degrees C., while under a nitrogen blanket and agitation. Three feeds identified herein as A, B, and C are next gradually and simultaneously added to the vessel over a period of two hours while the contents of the vessel are maintained at reflux conditions. Feed A consists of a mixture of 232.0 g isobornyl methacrylate, 696.0 g styrene, 464.0 g butyl methacrylate, 464.0 g methyl methacrylate, and 464.0 g gamma-methacryloxypropyltrimethoxysilane. Feed B consists of a mixture of 264.0 g of butyl acetate and 116 g 2,2'-azobis-(2-methyl butane nitrile) available as VAZO-67 from E.I. DuPont de Nemours and Company. Feed C consists of 132.0 g butyl acetate and 116.0 g gamma-mercaptopropyltrimethoxysilane. After the addition of the three feeds A, B, and C is complete, a mixture of 22 g butyl acetate and 9.28 g VAZO-67 is added all at once to the vessel and the contents of the vessel held at reflux for 1 hour. Next, another mixture of 22 g butyl acetate and 9.28 g of the VAZO-67 is added all at once to the vessel and the contents of the vessel thereafter held at reflux for an additional 1½ hours after which period heating is discontinued and the contents of the vessel allowed to cool to room temperature.

The resultant product is an addition interpolymer suitable for the method of the invention.

The resultant product has a theoretical total solids content of 72.5 percent by weight, an experimentally determined total solids content at 150 degrees C. for 1 hour of 70.6 percent by weight, a viscosity of 13.7 Stokes, an acid value of 0, a color value of 1, and a peak molecular weight of the addition interpolymer of 3651 as determined by gel permeation chromatography using a polystyrene standard. Analysis of the resultant product shows a content of butyl methacrylate of 0.41 percent by weight, a content of isobornyl methacrylate of 0.22 percent by weight and a content of styrene of 0.05 percent by weight.

## EXAMPLE 7

The following monomers are used to make an addition interpolymer for the clearcoating composition E of Example 9:

|                        | Percent by Weight |
|------------------------|-------------------|
| Isobornyl methacrylate | 40.0              |
| Styrene                | 20.0              |
| Methyl methacrylate    | 20.0              |
| Gamma-methacryloxy-    | 20.0              |
| propyltrimethoxysilane |                   |

A 4-neck flask equipped with condenser, stirrer, thermometer, 3 dropping funnels, and means for maintaining a nitrogen blanket is charged with 440.0 g of butyl acetate and heated to reflux, about 125 degrees C., while under a nitrogen blanket and agitation. Three feeds identified herein as A, B, and C are next gradually and simultaneously added to the vessel over a period of two hours while the contents of the vessel are maintained at reflux conditions. Feed A consists of a mixture

of 928.0 g isobornyl methacrylate, 464.0 g styrene, 464.0 g methyl methacrylate, and 464.0 g gamma-methacryloxypropyl trimethoxysilane. Feed B consists of a mixture of 264.0 g of butyl acetate and 116 g 2,2'-azobis-(2-methyl butane nitrile) available as VAZO-67 from E.I. DuPont de Nemours and Company. Feed C consists of 132.0 g butyl acetate and 116.0 g gamma-mercaptopropyl trimethoxysilane. After the addition of the three feeds A, B, and C is complete, a mixture of 22 g butyl acetate and 9.28 g VAZO-67 is added all at once to the vessel and the contents of the vessel held at reflux for 1 hour. Next, another mixture of 22 g butyl acetate and 9.28 g of the VAZO-67 is added all at once to the vessel and the contents of the vessel thereafter held at reflux for an additional 1½ hours after which period heating is discontinued and the contents of the vessel allowed to cool to room temperature.

The resultant product is an addition interpolymer suitable for the method of the invention.

The resultant product has a theoretical total solids content of 72.5 percent by weight, an experimentally determined total solids content at 150 degrees C. for 1 hour of 68.6 percent by weight, a viscosity of 13.2 Stokes, an acid value of 0.0, a color value of 2, and a peak molecular weight of the addition interpolymer of 3119 as determined by gel permeation chromatography using a polystyrene standard. Analysis of the resultant product shows a content of methyl methacrylate of 0.56 percent by weight, a content of isobornyl methacrylate of 1.69 percent by weight and a content of styrene of 0.02 percent by weight.

#### EXAMPLE 8

The following monomers are used to make a comparative silane addition interpolymer for use in the comparative clearcoating composition F of Example 9.

|                                          | Percent by Weight |
|------------------------------------------|-------------------|
| Methyl methacrylate                      | 40.0              |
| Styrene                                  | 25.0              |
| Gamma-methacryloxypropyltrimethoxysilane | 25.0              |
| 2-Ethylhexyl methacrylate                | 10.0              |

A 4-neck flask equipped with condenser, stirrer, thermometer, 3 dropping funnels, and means for maintaining a nitrogen blanket is charged with 448.0 g of butyl acetate, 192.0 g of VM & P Naphtha and 128.0 g of toluene and heated to reflux while under a nitrogen blanket and agitation. Three feeds identified herein as A, B, and C are next gradually and simultaneously added to the vessel over a period of two hours while the contents of the vessel are maintained at reflux conditions. Feed A consists of a mixture of 768.0 g methyl methacrylate, 480.0 g styrene, 480.0 g gamma-methacryloxypropyl trimethoxysilane and 192.0 g 2-ethylhexyl methacrylate. Feed B consists of a mixture of 224.0 g of butyl acetate and 96 g 2,2'-azobis-(2-methyl butane nitrile) available as VAZO-67 from E.I. DuPont de Nemours and Company. Feed C consists of 224.0 g butyl acetate and 96.0 g gamma-mercaptopropyl trimethoxysilane. After the addition of the three feeds A, B, and C is complete, a mixture of 32.0 g butyl acetate and 7.68 g VAZO-67 is added all at once to the vessel and the contents of the vessel held at reflux for 1 hour. Next, another mixture of 32 g butyl acetate and 7.68 g of the VAZO-67 is added all at once to the vessel and the contents of the vessel thereafter held at reflux for an

additional 1½ hours after which period heating is discontinued and the contents of the vessel allowed to cool to room temperature.

The resultant product is a comparative silane addition interpolymer.

The resultant product has a theoretical total solids content of 60.0 percent by weight, an experimentally determined total solids content at 150 degrees C. for 1 hour of 58.0 percent by weight, a viscosity of 1.35 Stokes, an acid value of 0.2, a color value of 1-, and a peak molecular weight of the silane addition interpolymer of 3776 as determined by gel permeation chromatography using a polystyrene standard. Analysis of the resultant product shows a content of methyl methacrylate of 0.65 percent by weight, a content of 2-ethylhexyl methacrylate of 0.53 percent by weight and a content of styrene of 0.04 percent by weight.

#### EXAMPLE 9

This example illustrates advantages when acrylic silane addition interpolymers prepared from isobornyl methacrylate are utilized in clear topcoating (clearcoating) compositions applied over a basecoating composition in a "color plus clear" application.

(a) The formulations of the basecoating composition and clear coating compositions are as set forth in the following TABLES 1 and 2 respectively.

TABLE 1

| Basecoating Composition                   | Weight (grams) |
|-------------------------------------------|----------------|
| Methyl ethyl ketone                       | 20.5           |
| Butyl acetate                             | 36.9           |
| Diethylene glycol monobutyl ether acetate | 10.0           |
| Organoclay <sup>1</sup>                   | 0.9            |
| UV absorber <sup>2</sup>                  | 0.9            |
| Triethylorthoformate                      | 4.3            |
| Flow control agent <sup>3</sup>           | 0.3            |
| Pattern control agent <sup>4</sup>        | 40.0           |
| Acrylic silane solution <sup>5</sup>      | 83.6           |
| Pigment paste <sup>6</sup>                | 52.6           |

<sup>1</sup>Available as BENTONE SD-2 from NL Industries, Inc..

<sup>2</sup>Available from Ciba-Geigy Corp. as TINUVIN 328.

<sup>3</sup>Available as BYK 300 from BYK Mallinckrodt Chem. Produkte GmbH.

<sup>4</sup>A dispersion of organic polymer microparticles at 44 percent by weight solids in 56 percent by weight of a solvent mixture (containing 1.19 percent toluene, 2.67 percent VM & P naphtha, 6.91 percent butyl acetate, 26.95 percent ISOPAR E from EXXON Corp., and 62.93 percent heptane). The dispersion of organic polymer microparticles is prepared from 139.9 pbw of heptane, 59.9 pbw of ISOPAR E from EXXON Corp., 147.2 pbw of methylmethacrylate, 7.6 pbw of glycidylmethacrylate, 37.6 pbw of a dispersion stabilizer solution; 0.447 pbw of ARMEEN DMCD (dimethyl cocoamine), 1.081 pbw of VAZO 67 initiator, 1.592 pbw of n-octyl mercaptan, and 4.626 pbw of methacrylic acid. The dispersion stabilizer solution contained 40 percent by weight solids and 60 percent by weight of a mixture of solvents. The dispersion stabilizer is a polymer prepared by graft polymerizing 49.5 percent by weight of a reaction product of 10.8 percent by weight of glycidyl methacrylate and 89.2 percent by weight of 12-hydroxystearic acid, with 45.4 percent by weight of methylmethacrylate and 4.2 percent by weight of glycidyl methacrylate, wherein the resulting copolymer product containing pendant epoxy groups is reacted with 0.9 percent by weight of methacrylic acid. The mixture of solvents of the dispersion stabilizer solution contains 68.5 percent by weight of butylacetate, 26.3 percent by weight of VM & P naphtha, and 5.2 percent by weight of toluene. The dispersion of organic polymer microparticles is prepared according to the teachings of U.S. Pat. No. 4,147,688 hereby incorporated by reference.

<sup>5</sup>As made in Example 2.

<sup>6</sup>Prepared by combining 71.5 pbw of aluminum flake pigment, 41.9 pbw butyl acetate and 90.7 pbw of an acrylic polyol having a peak molecular weight of between 18,000 and 20,000 and a Gardner-Holdt viscosity of Y- (prepared from 30.0% by weight methyl methacrylate, 25.0% by weight styrene, 19.0% by weight butyl methacrylate, 12.0%

TABLE 1-continued

by weight 2-ethylhexyl acrylate and 14.0% by weight 2-hydroxyethyl acrylate).

TABLE 2

| Clearcoating Composition           | Weight (grams) |                |       |       |       |
|------------------------------------|----------------|----------------|-------|-------|-------|
|                                    | A              | B              | C     | D     | E     |
| Product of Example 3               | 137.5          | 0              | 0     | 0     | 0     |
| Product of Example 4               | 0              | 137.5          | 0     | 0     | 0     |
| Product of Example 5               | 0              | 0              | 137.5 | 0     | 0     |
| Product of Example 6               | 0              | 0              | 0     | 137.5 | 0     |
| Product of Example 7               | 0              | 0              | 0     | 0     | 137.5 |
| Cellulose acetate butyrate         | 1.0            | 1.0            | 1.0   | 1.0   | 1.0   |
| Butyl acetate                      | 43.2           | 43.2           | 43.2  | 43.2  | 43.2  |
| UV absorber <sup>1</sup>           | 2.0            | 2.0            | 2.0   | 2.0   | 2.0   |
| Polysiloxane solution <sup>2</sup> | 0.6            | 0.6            | 0.6   | 0.6   | 0.6   |
| Flow control agent <sup>3</sup>    | 0.6            | 0.6            | 0.6   | 0.6   | 0.6   |
| Flow control agent <sup>4</sup>    | 0.2            | 0.2            | 0.2   | 0.2   | 0.2   |
| Triethylorthoformate               | 5.0            | 5.0            | 5.0   | 5.0   | 5.0   |
| Dibutyl tin dilaurate              | 2.0            | 2.0            | 2.0   | 2.0   | 2.0   |
| Thinner <sup>5</sup>               | 40.5           | 40.5           | 40.5  | 40.5  | 40.5  |
| Total weight                       | 232.6          | 232.6          | 232.6 | 232.6 | 232.6 |
| Percent Solids                     | 43.0%          | 43.0%          | 43.0% | 43.0% | 43.0% |
| F (comparison)                     |                | G (comparison) |       |       |       |
| Product of Example 8               | 170.7          |                | 0     |       |       |
| Product of Example 2               | 0              |                | 148.6 |       |       |
| Cellulose acetate butyrate         | 1.0            |                | 1.0   |       |       |
| Butyl acetate                      | 10.0           |                | 32.1  |       |       |
| UV absorber <sup>1</sup>           | 2.0            |                | 2.0   |       |       |
| Polysiloxane solution <sup>2</sup> | 0.6            |                | 0.6   |       |       |
| Flow control agent <sup>3</sup>    | 0.6            |                | 0.6   |       |       |
| Flow control agent <sup>4</sup>    | 0.2            |                | 0.2   |       |       |
| Triethylorthoformate               | 5.0            |                | 5.0   |       |       |
| Dibutyl tin dilaurate              | 2.0            |                | 2.0   |       |       |
| Thinner <sup>5</sup>               | 40.5           |                | 85.7  |       |       |
| Total weight                       | 232.6          |                | 277.8 |       |       |
| Percent Solids                     | 43.0%          |                | 36.0% |       |       |

<sup>1</sup> Available from Ciba-Geigy Corp. as TINUVIN 328.

<sup>2</sup> The polysiloxane is available from DOW Corning Corporation as DC 200, 135 csk. Dissolved in xylene to give a 0.5 percent polysiloxane content.

<sup>3</sup> Available as BYK 300 from BYK Mallinckrodt Chem. Produkte GmbH.

<sup>4</sup> Available as MODAFLOW from Monsanto Industrial Chemicals Company.

<sup>5</sup> The thinner contains 23 percent butyl acetate, 6 percent ethyl acetate, 4 percent xylene, 25 percent VM & P naphtha, 24 percent toluene, 6 percent DOWANOL PM acetate from DOW CORNING Corp., and 11 percent HEXATE 100 from Shell Chemical Co., all percentages being by volume.

The basecoating composition (see TABLE 1) is reduced 150 percent by volume with a lacquer thinner available as DTL-105 from DITZLER Automotive Finishes, PPG INDUSTRIES, INC., (i.e., 1 part by volume basecoating composition to 1.5 parts by volume lacquer thinner). The basecoating composition is spray applied to 24 gauge cold rolled steel panels (treated with BONDERITE 40, primed with a primer surfacer available as DZL-32 from DITZLER Automotive Finishes, PPG INDUSTRIES, INC., and sanded with No. 400 grit paper) to form the basecoats. The basecoats are allowed to flash for 15 minutes at room temperature. Immediately thereafter, the clearcoating compositions (see TABLE 2 above) are spray applied to the basecoats to form clear topcoats (clearcoats).

The basecoats and clearcoats are allowed to moisture cure at room temperature for 24 hours under ambient atmospheric conditions to the dry film thicknesses of the basecoats and topcoats as set forth in the following TABLE 3. Some properties of the resulting cured composite basecoat/clearcoats are as set forth in TABLE 3. These properties are determined after 24 hours and 120 hours respectively from when the clearcoating compositions are applied to the basecoats. In TABLE 3 the left and right hand entries represented with a slash in be-

tween (as in 4B/B) mean the respective values for the property determined after 24 hours and 120 hours respectively. "DFT BC" means "dry film thickness in mils of the basecoat", and "DFT CC" means "dry film thickness in mils of the clearcoat". "DOI" means "distinctness of image" measured 24 hours after application of the clearcoating composition to the basecoat. A film having a high distinctness of image when viewed from a direction close to the normal to the surface and under, for example, a light fixture such as a fluorescent light fixture having a cross-hatch grid in front of the bulb, exhibits a reflected image of the lighted fixture in the film which appears clear and sharply distinct and seems to originate deep in the film. "Tg" means the calculated glass transition temperature in degrees C. for the acrylic silane interpolymer utilized in the clearcoating composition. "Gasoline soak" means resistance to deterioration by the composite film to soaking for 3 minutes in gasoline. For gasoline soak a rating of 1 means excellent; a rating of 1- means very good; and a rating of 2 means good.

TABLE 3

| Example | Degree Gloss | DOI | Tg  | Pencil Hardness |      | Gasoline Soak | DFT BC | DFT CC |
|---------|--------------|-----|-----|-----------------|------|---------------|--------|--------|
|         |              |     |     | 20              | 20   |               |        |        |
| A       | 87/87        | 65  | 110 | 4B/B            | 2/1  | 0.8           | 2.6    |        |
| B       | 91/91        | 70  | 105 | 4B/B            | 1/1  | 0.8           | 2.6    |        |
| C       | 92/91        | 70  | 100 | 4B/B            | 1-1/ | 0.8           | 2.5    |        |
| D       | 93/93        | 80  | 97  | 4B/B            | 1/1  | 0.8           | 2.6    |        |
| E       | 93/93        | 85  | 120 | 4B/B            | 1-1/ | 0.8           | 2.7    |        |
| F       | 91/92        | 55  | 87  | 4B/B            | 1/1  | 0.8           | 2.7    |        |
| (Comp.) |              |     |     |                 |      |               |        |        |
| G       | 91/91        | 60  | 70  | 4B/B            | 1/1  | 0.8           | 2.4    |        |
| (Comp.) |              |     |     |                 |      |               |        |        |

What is claimed is:

1. A method of coating a substrate comprising the steps of:
  - (A) coating a substrate with one or more applications of a pigmented basecoating composition containing a film-forming resin to form a basecoat; and
  - (B) coating said basecoat with one or more applications of a topcoating composition comprising
    - (a) an addition interpolymer containing at least one silicon atom directly bonded to a hydrolyzable group, said addition interpolymer derived from a mixture of copolymerizable ethylenically unsaturated monomers comprising an isobornyl group-containing monomer selected from the group consisting of isobornyl methacrylate, isobornyl acrylate and a mixture thereof; wherein the amount of said isobornyl group-containing monomer ranges from 10 percent to 60 percent by weight based on the total weight of said mixture of copolymerizable ethylenically unsaturated monomers; and
    - (b) an effective amount of a cure promoting catalyst.
2. A method of coating a substrate comprising the steps of:
  - (A) coating a substrate with one or more applications of a pigmented basecoating composition containing a film-forming resin to form a basecoat; and
  - (B) coating said basecoat with one or more applications of a topcoating composition comprising
    - (a) an addition interpolymer containing alkoxy silane groups and/or acyloxy silane groups, said addition interpolymer derived from the reaction

of a mixture of monomers wherein said mixture of monomers contains:

(i) one or more ethylenically unsaturated silicon-free monomers comprising an isobornyl group-containing monomer selected from the group consisting of isobornyl methacrylate, isobornyl acrylate and a mixture thereof; and

(ii) a copolymerizable ethylenically unsaturated silane monomer selected from the group consisting of an alkoxy silane monomer, an acyloxy silane monomer, and a mixture thereof;

wherein the amount of said isobornyl group-containing monomer ranges from 10 percent to 60 percent by weight based on the total weight of said mixture of monomers; and

(b) an effective amount of a cure promoting catalyst.

3. The method of claim 2 wherein the amount of said ethylenically unsaturated silicon-free monomers ranges from about 50 percent to about 95 percent by weight based on the total weight of said mixture of monomers, and the amount of said copolymerizable ethylenically unsaturated silane monomer ranges from about 5 to about 50 percent by weight based on the total weight of said mixture of monomers.

4. The method of claim 2 wherein said ethylenically unsaturated silicon-free monomers (i) comprise an alkyl acrylate, alkyl methacrylate, vinyl aromatic hydrocarbon or a mixture thereof.

5. The method of claim 4 wherein said alkyl acrylate and alkyl methacrylate contain from 1 to 12 carbon atoms in the alkyl group.

6. The method of claim 4 wherein said vinyl aromatic hydrocarbon is styrene, vinyl toluene, alpha-methylstyrene or a mixture thereof.

7. The method of claim 6 wherein said silane monomer is a (meth)acrylatoalkoxysilane monomer having from 1 to 4 carbon atoms in the alkoxy group.

8. The method of claim 7 wherein said (meth)acrylatoalkoxysilane monomer is gamma-methacryloxypropyltrimethoxysilane, gamma-methacryloxypropyltriethoxysilane, or a mixture thereof.

9. The method of claim 2 wherein said addition interpolymer of said topcoating composition has a peak molecular weight as determined by gel permeation chromatography of at least about 2,000.

10. The method of claim 9 wherein said addition interpolymer of said topcoating composition has a calculated glass transition temperature of at least about 25 degrees Celsius.

11. The method of claim 2 wherein said addition interpolymer of said topcoating composition has a peak molecular weight as determined by gel permeation chromatography ranging from about 2,000 to about 20,000 and has a calculated glass transition temperature of at least about 25 degrees Celsius.

12. The method of claim 11 wherein said mixture of monomers contains from about 70 percent to about 90 percent by weight of said ethylenically unsaturated silicon-free monomers (i), from about 10 percent to about 30 percent by weight of said copolymerizable ethylenically unsaturated silane monomer (ii), and from 40 percent to 20 percent by weight of said isobornyl group-containing monomer, based on the total weight of said mixture of monomers, and wherein said addition interpolymer of said topcoating composition has a cal-

culated glass transition temperature of from about 30 degrees Celsius to about 120 degrees Celsius.

13. The method of claim 9 wherein a mercaptoalkyl trialkoxysilane is used as a chain transfer agent in the reaction of said mixture of monomers.

14. A method of coating a substrate comprising the steps of:

(1) coating a substrate with one or more applications of a pigmented basecoating composition comprising an addition interpolymer containing at least one silicon atom directly bonded to a hydrolyzable group, said addition interpolymer derived from a mixture of copolymerizable ethylenically unsaturated monomers comprising an isobornyl group-containing monomer selected from the group consisting of isobornyl methacrylate, isobornyl acrylate and a mixture thereof; wherein the amount of said isobornyl group-containing monomer ranges from 10 percent to 60 percent by weight based on the total weight of said mixture of copolymerizable ethylenically unsaturated monomers,

to form a basecoat; and

(2) coating said basecoat with one or more applications of a topcoating composition comprising a film-forming resin to form a clear topcoat.

15. A method of coating a substrate comprising the steps of:

(a) coating a substrate with one or more applications of a pigmented basecoating composition comprising an addition interpolymer containing alkoxy silane groups and/or acyloxy silane groups, said addition interpolymer derived from the reaction of a mixture of monomers wherein said mixture of monomers contains:

(i) at least two ethylenically unsaturated silicon-free monomers one of which is an isobornyl group-containing monomer selected from the group consisting of isobornyl methacrylate, isobornyl acrylate and a mixture thereof; and

(ii) a copolymerizable ethylenically unsaturated silane monomer selected from the group consisting of an alkoxy silane monomer, an acyloxy silane monomer, and a mixture thereof, wherein the amount of isobornyl methacrylate ranges from 10 percent to 60 percent by weight based on the total weight of said mixture of monomers,

to form a basecoat; and

(b) coating said basecoat with one or more applications of a topcoating composition comprising a film-forming resin to form a clear topcoat.

16. The method of claim 15 wherein the amount of said ethylenically unsaturated silicon-free monomers ranges from about 50 percent to about 95 percent by weight based on the total weight of said mixture of monomers, and the amount of said copolymerizable ethylenically unsaturated silane monomer ranges from about 5 to about 50 percent by weight based on the total weight of said mixture of monomers.

17. The method of claim 15 wherein said ethylenically unsaturated silicon-free monomers (i) comprise an alkyl acrylate, alkyl methacrylate, vinyl aromatic hydrocarbon or a mixture thereof.

18. The method of claim 17 wherein said alkyl acrylate and alkyl methacrylate contain from 1 to 12 carbon atoms in the alkyl group.

19. The method of claim 17 wherein said vinyl aromatic hydrocarbon is styrene, vinyl toluene, alpha-methylstyrene or a mixture thereof.

20. The method of claim 17 wherein said silane monomer is a (meth)acrylatoalkoxysilane monomer having from 1 to 4 carbon atoms in the alkoxy group.

21. The method of claim 20 wherein said acrylatoalkoxysilane monomer is gamma-methacryloxypropyltrimethoxysilane, gamma-methacryloxypropyltriethoxysilane, or a mixture thereof.

22. The method of claim 15 wherein said addition interpolymer of said basecoating composition has a peak molecular weight as determined by gel permeation chromatography ranging from about 2,000 to about 20,000 and having a calculated glass transition temperature of at least about 25 degrees Celsius.

23. The method of claim 15 wherein said mixture of monomers contains from about 70 percent to about 90 percent by weight of said ethylenically unsaturated silicon-free monomers (i), from about 10 percent to about 30 percent by weight of said copolymerizable ethylenically unsaturated silane monomer (ii), and from 40 percent to 20 percent by weight of said isobornyl group-containing monomer based on the total weight of said mixture of monomers, and wherein said addition 10 interpolymer of said basecoating composition has a calculated glass transition temperature of from about 30 degrees Celsius to about 120 degrees Celsius.

24. The method of claim 23 wherein a mercaptoalkyl trialkoxysilane is used as a chain transfer agent in the 15 reaction of said mixture of monomers.

\* \* \* \* \*